

## UNITED STATES PATENT OFFICE

2,213,972

## ARTIFICIAL FIBER SUITABLE FOR YIELDING DYEINGS FAST TO FULLING

Arthur von Weinberg, Frankfort-on-the-Main,  
 Hanns Rein, Bad Homburg vor der Höhe, and  
 Otto Eisenhut, Heidelberg, Germany, assignors  
 to I. G. Farbenindustrie Aktiengesellschaft,  
 Frankfort-on-the-Main, Germany

No Drawing. Application September 17, 1937,  
 Serial No. 164,334. In Germany November 29,  
 1935

9 Claims. (Cl. 8—22)

Our U. S. application Ser. No. 113,012, filed November 27, 1936, relates to artificial fibers suitable for yielding dyeings fast to fulling and process of making same.

5 Our present invention is a continuation in part of the said application and relates likewise to artificial fibers suitable for yielding dyeings fast to fulling and process of making same.

In employing all types of artificial fibers in 10 admixture with wool, particularly for the manufacture of woven materials which must have an excellent resistance to wear, such as for example military cloth, gentlemen's suitings and so on, the tinctorial properties of the artificial fibers 15 involve great difficulties because they are quite different from those of wool. Hitherto when the material was intended to exhibit particular resistance properties it was necessary to dye the two different fibers by separate dyeing methods.

20 Some other dyeing methods were disadvantageous because the dye-baths could not be exhausted and dyestuff was lost.

Various proposals have already been made for 25 treating the artificial fibers by the addition of such compounds containing nitrogen as are capable of reacting with acid dyestuffs such as for example albuminous compounds, or for incorporating such compounds into the fibers. It has been found however, that fibers thus treated can only be weakly dyed, in particular more weakly than the wool contained in the above mixed textile fabrics. Alternatively, by employing the usual dyeing methods for wool, during the dyeing process at elevated temperatures or 35 during the fulling process the artificial fibers give up the dyestuff first absorbed to the admixed wool. The latter occurs particularly easily when the fibers have only subsequently been treated with the nitrogenous compounds.

40 Now we have found that artificial fibers suitable for yielding dyeings fast to fulling are obtained by incorporating to artificial fibers during their process of manufacture either single or as mixtures nitrogenous bases which contain 45 on the one side an aliphatic radicle of a long chain of carbon atoms, on the other side the radicle of an aliphatic polyamine. Such nitrogenous bases are capable of forming with dyestuffs of the type of the so-called metachrome-dyestuffs (i. e., dyestuffs which may be dyed and chromed at the same time, f. i., in a single bath by means of the metachrome-mordant, f. i., ammoniumbichromate), in a neutral bath in the presence of the metachrome-mordant and without the addition of acid, complex compounds

which are fast to boiling. Artificial fibers of the aforesaid kind may be mixed with wool and such mixtures may be dyed according to the single-bath process by means of metachrome dyestuffs with the production of equal dyeings, 5 fast to fulling.

As nitrogenous bases which are to be incorporated in the artificial fibers there may be named particularly the condensation product of halogenation products of hard paraffin (i. e., the well known technical product of 54 to 56° melting point, consisting of a mixture of saturated hydrocarbons ranging from tetracosan  $C_{24}H_{50}$  to heptacosan  $C_{27}H_{56}$ , cf. Ullmann, Enzyklopädie der technischen Chemie, second edition (1912), vol. 2, 10 page 611 ff.) with polyalkylene polyamines. As polyalkylene polyamines there may be used for the purpose of the present invention particularly the reaction products of ammonia with alkylene polyhalogenides like ethylene dichloride, 15 ethylene dibromide, propylene dichloride, the halogeno derivatives of glycerine, butylene dichloride and other similar halogenides. The polyalkylene polyamines thus obtained usually consist of several components of different molecular weight, for example of dialkylene triamines, trialkylene tetramines and so on. For the present invention particularly the crude mixture of these products may be used as starting 20 material.

The aforesaid nitrogenous bases may be incorporated single or a plurality thereof, in a given case in admixture with a suitable aliphatic polyamine which has not been subjected to the above condensation reaction.

When the artificial fiber is a viscose material, it is advantageous to employ such material as is similar to copper silk in its properties, for instance an artificial fiber which is obtained by treatment with agents capable of removing water. In some cases it is of an advantage to subject the fibers before the dyeing process to a cleansing operation using reducing agents such as for example hydrosulfite.

In order to further illustrate our invention the 45 following examples are given, the parts being by weight and all temperatures in centigrade degrees. However, we wish it to be understood that our invention is not limited to the particular products nor reaction conditions mentioned therein.

## Example 1

A viscose material which is prepared by employing a viscose ripened below the usual ripeness is mixed before spinning in a suitable mix-

ing vessel for instance in a Werner-Pfleiderer apparatus with 3% of its weight (with respect to the content of cellulose) of an aqueous suspension of a base obtained by condensing tri-chloro-hard paraffine with polyethylene-poly-amine. (In order to prepare the above trichloro-derivative hard paraffine of 54 to 56° C. melting point has been chlorinated by introducing chlorine at temperatures beginning at 80° and ending at 50-60°, until an increase in weight corresponding to the entrance of three chlorine atoms has taken place (cf. U. S. Patent 1,948,924). The above polyethylene polyamine mixture has been prepared by acting with aqueous ammonia on ethylene chloride and removing the fractions, boiling under 10 mm. pressure up to 220°, by distillation. The residue thus obtained is a viscous brown liquor). The viscose material is spun, acidified, washed and drawn through a hot hydrosulfite bath in order to cleanse it. Then it is washed again and finally treated with alcohol in accordance with the process of our U. S. Patent 2,109,306, February 22, 1938. The fiber thus obtained is distinguished by a wool-like appearance. A textile fabric obtained from the new fiber mixed with wool may be dyed for example with Metachrome Brilliant Blue 8RL (Schultz, Farbstofftabellen, 7th edition, supplement, vol. I, page 111) whereby equal dyeings are obtained, fast to fulling.

*Example 2*

In a viscose material of the usual degree of ripeness 2% of its weight of the same base as used in Example 1 are incorporated in the above described manner and the viscose is spun in the usual manner. The well washed product is treated at about 50° with a solution of hydrogen peroxide of 1% strength whereby a light fibrous material is obtained, even when a remarkably colored base is used.

A textile fabric obtained from the new fiber may be mixed with wool and dyed for example with Metachrome-olive-brown (Schultz, Farbstofftabellen, 7th edition, No. 142) or Metachrome-brown CG (l. c., vol. II, page 146) whereby intense and equal dyeings are obtained, entirely fast to fulling.

*Example 3*

50 In a viscose material as used in Example 1 immediately while dissolving it or thereafter 4% of its weight of a mixture are incorporated, which consists in the same proportions of the base used in the foregoing examples, of the condensation product of pentachlorohard paraffine (cf. U. S. Patent 1,948,924) and polyethylenopolyamine and of a mixture of polyethylenopolyamine itself (cf. Example 1), from which the fractions boiling in vacuo of 10 mm. until 220° have been previously removed by distillation.

Then the viscose material is worked up as described in Example 1, but not treated with hydrosulfite, rather at 50° with a hydrogen peroxide solution of 1% strength.

65 A textile fabric obtained from the new fiber exhibits a very wool like character and yields, when dyed according to the meta chrome dyeing process for instance with Alizarine blue black

B (Schultz, l. c. No. 1195) or Chromoxane pure blue (l. c. vol. II, page 59) dyeings of practically the same fastness to light and fulling as when pure wool has been dyed with the same dyestuffs.

*Example 4*

A copper-ammonia cellulose spinning solution as usual for spinning copper silk is mixed in a good mixing vessel with 2% of its weight (related to the cellulose content of the solution) of the condensation product as described in Example 1. Then the solution is shortly deaerated and spun in a spinning funnel into water, soured, cut up and worked up as usual. In a given case to the after-treating bath hydrogen peroxide may be added. In this manner a textile fabric is obtainable which may be dyed in admixture with wool with a suitable dyestuff, for instance a metachrome dyestuff, thus yielding dyeings, fast to fulling.

We claim:

1. Artificial fibers prepared from rayon spinning solutions selected from the group consisting of viscose and cuprammonia solutions which fibers contain nitrogenous bases having an aliphatic radicle of a long chain of carbon atoms and a radicle of a polyalkalene polyamine, the fibers being suitable for yielding dyeings fast to fulling.

2. Artificial fibers prepared from rayon spinning solutions selected from the group consisting of viscose and cuprammonia solutions which fibers contain a condensation product obtained by condensing a tri-chlorinated derivative of hard paraffine with a polyethylene polyamine, the fibers being suitable for yielding dyeings fast to fulling.

3. Artificial fibers prepared from a viscose of a low degree of ripeness which fibers contain a condensation product of a tri-chlorinated hard paraffine with a polyethylene polyamine obtained by acting with aqueous ammonia on ethylene dichloride and removing the fractions boiling under 10 mm. pressure up to 220° by distillation, the fibers being suitable for yielding dyeings fast to fulling.

4. Artificial fibers in accordance with claim 1 which are dyed by a metachrome dyestuff.

5. Artificial fibers in accordance with claim 2 dyed with a metachrome dyestuff.

6. An artificial fiber in accordance with claim 3 dyed with a metachrome dyestuff.

7. Mixed fibers of wool and artificial fibers in accordance with claim 1, which are dyed by means of metachrome dyestuffs with the production of equal dyeings, fast to fulling.

8. Mixed fibers of wool and artificial fibers in accordance with claim 2, which are dyed by means of metachrome dyestuffs with the production of equal dyeings fast to fulling.

9. Mixed fibers of wool and an artificial fiber in accordance with claim 3 which are dyed by means of metachrome dyestuffs with the production of equal dyeings fast to fulling.

ARTHUR VON WEINBERG.  
HANNS REIN.  
OTTO EISENHUT.